

Nov. 3, 1959

W. J. L. KEARNS

2,911,453

METHOD OF STARTING UP A DEHYDROGENATION PROCESS

Filed April 23, 1956



*Inventor*  
William J. L. Kearns  
by  
Stevens, Davis, Miller & Kafer  
his attorneys

1

2,911,453

## METHOD OF STARTING UP A DEHYDRO- GENATION PROCESS

William J. L. Kearns, Corunna, Ontario, Canada, assignor to Polymer Corporation Limited, Sarnia, Ontario, Canada, a corporation of Canada

Application April 23, 1956, Serial No. 579,793

4 Claims. (Cl. 260—680)

This invention relates to a process for the dehydrogenation of olefinic hydrocarbons, particularly monoolefins containing at least four carbon atoms in the olefinic chain. More particularly it relates to a method of commencing the dehydrogenation reaction and still more particularly it relates to a method for the "start-up" of the reaction.

In this specification the term "start-up" is intended to mean those series of steps which serve to raise the temperature of the dehydrogenation catalyst to the normal dehydrogenation temperature.

The catalysts envisaged in the process of the present invention are those which, during the process of their manufacture into the commercially acceptable form become admixed with a combustible lubricant, which must subsequently be removed. The better-known of such catalysts are those in which the active ingredient is calcium nickel phosphate. The most widely used catalyst of this type is the calcium nickel phosphate-chromium oxide catalyst disclosed in United States Patent No. 2,442,320 issued May 25, 1948 to Andrew J. Dietzler et al. This particular catalyst is in the form of pellets. During the process of the manufacture of such pellets they become admixed with combustible lubricant, such as graphite, which must subsequently be removed in order that the dehydrogenation reaction may proceed.

In order to remove the combustible lubricant from the catalyst, it is necessary to heat the catalyst in the presence of steam and a controlled amount of oxygen or oxygen-containing gas, e.g. air so that such combustible lubricant burns off at a sufficiently slow rate that it does not damage the catalyst.

Catalysts of the type used in the present invention for the dehydrogenation of monoolefins conventionally require superheated steam in the process. To avoid wetting the catalyst during "start-up," the charged reactors have, in the past, used the following method of "start-up":

The charged reactors are warmed above the condensation point of steam by recirculating fuel gas through heaters and then through the catalyst beds. In order that fuel gas and oxygen are not intermixed within explosive limits, the large reactors, furnaces, and connecting equipment are usually purged with an inert gas, which is essentially nitrogen and carbon dioxide. This purging operation usually requires as much as 36 hours time during the start-up procedure, since most plants are not capable of producing large quantities of such infrequently used gas. When the oxygen content of the effluent is less than about 0.5%, the inert gas is displaced with fuel gas and recirculation is then established between the furnaces and the reactors. When the catalyst beds are heated to a temperature greater than 212° F., preferably

2

400—600° F. the circulation of fuel gas is terminated, and superheated steam is added. The steam is passed through the catalyst bed until it reaches a temperature of about 900 to 1150° F. at which time a controlled amount of oxygen or oxygen-containing gas, e.g. air, is added together with the steam for the purpose of oxidizing the carbonaceous material from the catalyst.

The entire process is lengthy and costly, firstly, because of the fact that fuel gas is used to heat the catalyst. Such fuel gas creates a fire hazard in that there is possible furnace damage from tube leakage of fuel gas into the combustion zones. Secondly, because of the amount of inert gas needed to purge the reactors, the purging operation is time consuming.

15 It is, therefore, an object of the invention to effect a start-up of the dehydrogenation in such a manner that a minimum of time is wasted.

16 It is a further object of this invention to provide a safer method of effecting such start-up.

20 These and other objects are achieved in the process of commencing a dehydrogenation reaction using new catalyst, in the form of pellets which contain a combustible lubricant in the improvement which comprises effecting such start-up by passing hot air at a maximum temperature of about 600° F. through such catalyst until the minimum temperature of such catalyst bed is at least slightly higher than the temperature at which steam condenses upon such catalyst. Subsequent heating of the air-heated catalyst to its normal operating temperature includes passing superheated steam through the catalyst in order to heat such catalyst to the required operating temperature. A controlled amount of air is then admixed with the steam and passed through the catalyst to oxidize said combustible lubricant.

25 35 More particularly, the invention resides in the process of effecting the start-up of a new calcium nickel phosphate-chromium oxide catalyst, in the form of pellets which contain graphite, in the improvement which comprises effecting such start-up by passing hot air through

40 such catalyst until the minimum temperature of the entire catalyst bed is at least 225° F., and, for safety purposes, is at a maximum temperature of 600° F. Subsequent heating of the air-heated catalyst to its normal operating temperature includes passing superheated steam through such catalyst, in order to heat said catalyst to the required operating temperature. A controlled amount of air is then admixed with the steam and passed through the catalyst in order to oxidize the graphite therefrom.

45 50 The minimum and maximum temperatures to which the catalyst bed is heated by means of the hot air only, are subject to slight variations, depending upon the safety factor desired. For example, the minimum temperature is set by the condition that the presence of free water on the catalyst is to be avoided. Hence, theoretical considerations would require a minimum temperature of 212° F. However, in order to avoid the danger that certain areas of the catalyst bed may be at a temperature below the temperature indicated by the thermocouples used to measure the temperature, it is advisable to operate at a minimum temperature of 225° F. Similarly, examples to be given below indicate the graphite burns off the catalyst at temperatures greater than 885° F. Nevertheless, it is theoretically possible for the graphite to ignite at temperature lower than 885° F., and a slight amount of burning would spread uncontrolled over a large amount of catalyst, thereby resulting in making un-

suitable for the dehydrogenation the catalyst so ignited. Hence, it is advisable to impose a maximum limit on the temperature to which the catalyst is raised by means of the hot air. The maximum temperature contemplated in the present invention is 600° F., but, higher temperatures may be used if so desired. However, at temperatures in excess of 600° F., the higher the temperature, the greater is the danger of uncontrolled combustion of the combustible lubricant on the catalyst.

Pilot plant and commercial scale operations were carried out to determine the optimum temperature for the air start-up procedure.

The Pilot Plant experiments to determine a safe air temperature for purposes of heating up beds of new calcium nickel phosphate-chromium oxide catalyst was divided into two stages; the first stage consisted of four experiments, the first two involving the use of a modified Pilot Plant reactor which contained approximately 160 lbs. of calcium nickel phosphate-chromium oxide catalyst, while the other two experiments were carried out in the normal Pilot Plant isothermal reactor containing approximately 335 grams of calcium nickel phosphate-chromium oxide catalyst; the second stage involved the use of larger samples of the calcium nickel phosphate-chromium oxide catalyst, using the apparatus shown diagrammatically in Fig. 1. The commercial scale operations were performed in two experiments using the standard amounts of catalyst, and with a flow of air of 18,000 lb./hr.

The first stage of the Pilot Plant experiments consisted of passing preheated air through the catalyst beds at increasingly higher temperatures and determining whether any graphite was burned off the catalyst by measuring the carbon dioxide content of the reactor effluent gases.

#### EXAMPLE I

The temperature of the heated air passing through a bed of 160 lbs. of calcium nickel phosphate-chromium oxide catalyst was raised progressively to a maximum of 645° F. During the run, the catalyst pellets at the top of the bed attained a temperature of 585° F. and pellets at a depth of one foot attained a temperature of 482° F. CO<sub>2</sub> analysis on the reactor effluent indicated that no graphite was being burned off the catalyst. On visual inspection at the end of the run, the catalyst appeared exactly the same as new calcium nickel phosphate-chromium oxide catalyst from the same lot.

#### EXAMPLE II

The temperature of the heated air passing through a bed of 169 lbs. of calcium nickel phosphate-chromium oxide catalyst was raised progressively to a maximum of 604° F. During the run, the catalyst pellets at the top of the bed attained a temperature of 596° F. and pellets at a depth of one foot attained a temperature of 541° F. CO<sub>2</sub> analysis on the reactor effluent indicated that no graphite was being burned off the catalyst. On visual inspection at the end of the run, the catalyst appeared exactly the same as new calcium nickel phosphate-chromium oxide catalyst from the same lot. Carbon analysis on the experimental calcium nickel phosphate-chromium oxide catalyst and new calcium nickel phosphate-chromium oxide catalyst revealed no difference in carbon content.

#### EXAMPLE III

Air was passed for three hours over a 333 gm. bed of calcium nickel phosphate-chromium oxide catalyst which was heated to 750° F.

CO<sub>2</sub> analysis on the reactor effluent indicated that no graphite was being burned off the catalyst. On visual inspection at the end of the run, the catalyst appeared exactly the same as the original new calcium nickel phosphate-chromium oxide catalyst.

#### EXAMPLE IV

Air was passed through a 334 gm. bed of calcium nickel phosphate-chromium oxide catalyst which was heated for successive three hour periods to 525° F., 705° F., 885° F., 1065° F. and 1245° F. CO<sub>2</sub> analysis on the reactor effluent showed a net increase above the temperature of 885° F. indicating that graphite was being burned off the catalyst. On visual inspection at the end of the run, the catalyst appeared completely burned off.

These four experiments indicate that the calcium nickel phosphate-chromium oxide catalyst may be preheated in the presence of air to a temperature below 850° F. They show that the graphite on the catalyst starts to burn off at temperatures above 850° F.

For the second stage of the Pilot Plant work, the apparatus shown diagrammatically in the drawing was used.

In the drawing it is seen that the reactor 1 consists of a drum containing a bed of catalyst 2 between upper and lower screens 3. The lower screen also rests upon fire bricks 4. Within the reactor are thermocouples 5, 6 and 7. Thermocouple 5 is for the purpose of measuring the air temperature just above the catalyst. Thermocouple 6 is for the purpose of measuring the catalyst temperature at about 1 1/4" below the surface of the catalyst bed. Thermocouple 7 is for the purpose of measuring the catalyst temperature at a distance of about 10 1/4" below the surface of the catalyst. The various temperatures were recorded using a Braun potentiometer-type multipoint recorder (not shown), range 32° F.-572° F. For temperatures above 572° F., a portable potentiometer box (also not shown) was substituted for the Braun multipoint recorder, and measurements were recorded by the operator. High pressure air is first passed through an air filter 8, through a pressure reducing valve 9 and rotameter 10 to the electric steam superheater 11. It is then passed through a 150 p.s.i. steam heated water evaporator 12, and subsequently to a third preheater 13. It then passes through 1" pipe 14 to the reactor 1, and it is admitted to the reactor by means of a nozzle 15 which consists of 8 1/4" holes drilled in a cap which covers the pipe 14 immediately within the reactor 1. Exit air then is passed through coolers 16 and 17. It was found that air temperatures as high as 650° F. were attained at a flow rate of 19.3 s.c.f.m. (calculated at 14.7 p.s.i. absolute and 70° F.). This represented 435 v./hr. per unit volume of catalyst and was the greatest air flow possible without increasing the size of the supply pipe lines.

During the operation, measurement of the carbon dioxide content of the air entering and leaving the reactor was made using the Orsatz caustic bubbler technique.

#### EXAMPLE V

The catalyst drum was loaded with 169 lb. of new calcium nickel phosphate-chromium oxide catalyst. With the furnace temperature set initially at 212° F. and eventually at 1200° F., air was passed over the catalyst at 35 v./v./hr. The maximum air temperature attained was 178° F. and the maximum catalyst temperature at the top of the reactor was 147° F. After 21 hours of operation certain changes were made in the air heating system and the air temperature attained with an air flow of 35 v./v./hr. was 217° F. When it was noticed that a brief reduction in air flow, to approximately 20 v./v./hr., was accompanied by a sharp decrease in temperature, the air flow was increased to 50 and then to 65 v./v./hr. and increases noticed in all temperatures.

After about 29 hours of operation the experiment was discontinued during a weekend shutdown and the catalyst temperature decreased from 180° F. to 80° F.

When the experiment was recommenced, irregularities were noticed in the temperature records for the first 30 minutes of operation. This was thought to be due to a

surge of very hot air from the furnace which had been heated to 1200° F.

The air rate was increased progressively from 35 v./v./hr. to 65, 87, 110, 140 and 187 v./v./hr. and increases were noted in both air and catalyst bed temperatures. An air temperature of 575° F. was achieved and the catalyst temperature increased to 520° F. at the top of the reactor and 250° F. at the bottom of the reactor.

The air rate was still further increased to 355 and then to 435 v./v./hr. A maximum temperature of 650° F. for the air was observed but it was not possible to maintain this temperature because certain physical limits of the apparatus used were reached. However, maximum catalyst temperatures of 590° F. at the top of the bed and 480° F. at the bottom of the bed were attained and maintained for several hours.

During the course of the experiment, the CO<sub>2</sub> content of the air effluent was measured at 30 minute intervals and was found to vary from nil to 1.7%. Suspicion that the high CO<sub>2</sub> readings were not realistic, lead to a check of the CO<sub>2</sub> content of the inlet air. In general these values were very close, almost within experimental error, to the values for the effluent air. With each increase in air flow a momentary increase in CO<sub>2</sub> content was observed.

After an interval of 7 days the experiment was discontinued and approximately 160 lb. of catalyst recovered. This catalyst was unchanged in physical appearance. Data, typical of that accumulated during this run is shown in Table I.

Table I

| Hours Operation | Air Flow, v./v./hr. | Air Temp., °F. | Bed Temperature |             | Percent CO <sub>2</sub> in air |     |
|-----------------|---------------------|----------------|-----------------|-------------|--------------------------------|-----|
|                 |                     |                | Top, °F.        | Bottom, °F. | In                             | Out |
| at start        |                     | 75             | 75              | 75          |                                |     |
| 6.5             | 37                  | 133            | 104             | 77          | 0.11                           |     |
| 11.5            | 37                  | 147            | 118             | 81          | 0.25                           |     |
| 16.5            | 37                  | 167            | 144             | 95          | 0.52                           |     |
| 21.5            | 37                  | 178            | 147             | 127         | nil                            |     |

Screens, etc. installed in heaters weekend shutdown and gradual cooling to 80° F.

|       |     |      |     |     |      |
|-------|-----|------|-----|-----|------|
| 32.0  | 37  | 118  | 133 | 80  | nil  |
| 37.0  | 37  | 217  | 137 | 127 | 0.12 |
| 42.0  | 87  | 400  | 235 | 136 | 0.75 |
| 47.0  | 187 | 560  | 433 | 142 | 0.71 |
| 52.0  | 187 | 570  | 480 | 155 | 0.77 |
| 57.0  | 187 | 568  | 487 | 206 | 0.13 |
| 62.0  | 140 | 575  | 500 | 239 | 0.25 |
| 66.0  | 187 | 675+ | 505 | 252 | 0.82 |
| 71.0  | 187 | 580  | 475 | 252 | 1.68 |
| 76.0  | 187 | 517  | 413 | 242 | 0.13 |
| 81.0  | 355 | 575+ | 532 | 270 | 0.30 |
| 86.0  | 355 | 575+ | 560 | 374 | 0.18 |
| 91.0  | 355 | 645  | 585 | 442 | 0.89 |
| 96.0  | 435 | 662  | 532 | 482 | 2.03 |
| 101.0 | 435 | 451  | 420 | 450 | 0.80 |
| 106.0 | 435 | 521  | 468 | 392 | 0.34 |
| 111.0 | 435 | 571  | 520 | 396 | 0.22 |

## EXAMPLE VI

The method of Example V was repeated and this time 160 lb. of new calcium nickel phosphate-chromium oxide catalyst was loaded into the drum. Operation was commenced using the conditions eventually found to be best in Example V, i.e., furnace temperatures set to 1200° F. to 1300° F. and air flow at 355 v./v./hr. Although difficulties were again experienced because of overloading the furnace circuit, the air temperature quickly increased to 500° F. During the initial warming up the maximum rate of temperature increase of the air was 3.5° F. per minute, the top of the catalyst bed 2.4° F. per minute, and the lower point in the catalyst bed

2.2° F. A delay of approximately 1 hour was noticed between the time of rapid temperature increase of the air and of the top of the catalyst bed. A further delay of approximately 4 hours elapsed before the lower temperature point recorded a rapid increase.

After about 24 hours of operation the air temperature reached 575° F., the top of the bed 564° F. and the bottom of the bed 520° F. These conditions were maintained for 16 hours and then the air flow was increased to 435 v./v./hr. The temperatures increased to a maximum of 604° F., 595° F. at the top of the bed and 540° F. at the bottom of the bed. The run was continued for an additional 18 hours at approximately these conditions.

As in the first run the CO<sub>2</sub> measurements were made on the air influx and efflux and the analysis indicated little, if any, net gain in CO<sub>2</sub>.

When the experiment was discontinued, approximately 155 lb. of catalyst was recovered and it could not be distinguished from new catalyst.

Typical data for this example are shown below in Table II.

Table II

| Hours Operation | Air Flow, v./v./hr. | Air Temp., °F. | Bed Temperature |             | Percent CO <sub>2</sub> in air |      |
|-----------------|---------------------|----------------|-----------------|-------------|--------------------------------|------|
|                 |                     |                | Top, °F.        | Bottom, °F. | In                             | Out  |
| 1               |                     | 355            | 260             | 185         | 153                            | 1.45 |
| 3               |                     | 355            | 419             | 345         | 153                            | 0.79 |
| 5               |                     | 355            | 490             | 465         | 252                            | 0.84 |
| 7               |                     | 355            | 510             | 490         | 400                            | 1.09 |
| 9               |                     | 355            | 490             | 480         | 445                            | 0.88 |
| 11              |                     | 355            | 489             | 455         | 445                            | 0.89 |
| 15              |                     | 355            | 480             | 463         | 430                            | 0.29 |
| 20              |                     | 355            | 555             | 537         | 480                            | 0.23 |
| 25              |                     | 355            | 575+            | 564         | 523                            | nil  |
| 30              |                     | 355            | 575+            | 565         | 523                            | 0.39 |
| 35              |                     | 355            | 575             | 560         | 521                            | 0.27 |
| 40              |                     | 435            | 604             | 596         | 507                            | 0.24 |
| 45              |                     | 435            | 582             | 570         | 541                            | 0.26 |
| 50              |                     | 435            | 591             | 582         | 541                            | 0.45 |
| 55              |                     | 435            | 588             | 577         | 537                            | 0.56 |
| 57              |                     | 435            | 587             | 574         | 535                            | 0.48 |

## EXAMPLE VII

Upon completion of the work described above, the additional air preheater was removed and the normal air heater was restored to its original service. A standard 25" tube of calcium nickel phosphate-chromium oxide catalyst (333 gms.) was loaded into the reactor tube and heated to 750° F. with air passing through it at 120 v./v./hr. The catalyst was maintained at this temperature for three hours and then removed for inspection. Again, there was no change in the physical appearance of the catalyst. The percent CO<sub>2</sub> in the air effluent varied from nil to 0.4 during the heating treatment. The weight of catalyst removed was 328 gms.

The observations for this example are recorded below in Table III.

Table III

| Hours Operation | Air Flow, v./v./hr. | Air Temp., No. 1 Thermo., °F. | Bed Temp., No. 2 Thermo., °F. | Percent CO <sub>2</sub> in air |      |
|-----------------|---------------------|-------------------------------|-------------------------------|--------------------------------|------|
|                 |                     |                               |                               | In                             | Out  |
| 1               |                     | 120                           | 770                           | 446                            | 0.36 |
| 2               |                     | 120                           | 762                           | 500                            | 0.42 |
| 3               |                     | 120                           | 762                           | 608                            | 0.39 |
| 4               |                     | 120                           | 752                           | 698                            | 0.11 |
| 5               |                     | 120                           | 752                           | 752                            | 0.13 |
| 6               |                     | 120                           | 752                           | 752                            | 0.19 |
| 7               |                     | 120                           | 788                           | 752                            | 0.30 |

## EXAMPLE VIII

Example VII was repeated under similar conditions. For this example 334 gms. of catalyst was charged to the

reactor and with air passing through it at 120 v.v./hr. the bed temperature was elevated for successive 3 hour periods to 525° F., 705° F., 885° F., 1065° F. and 1245° F. CO<sub>2</sub> measurements were made, as described above, on the air entering and leaving the reactor. At temperatures of 885° F. and above there appeared to be a net increase in the CO<sub>2</sub> present in the air from the reactor varying from 0.2 to 0.8%.

When the catalyst was removed after this experiment, all but approximately 1% of the pellets were completely burned off. The weight of catalyst removed was 324 gms. The typical data for this example are shown below in Table IV.

Table IV

| Hours Operation | Air Flow, v.v./hr. | Air Temp. No. 1 Thermo., ° F. | Bed Temp. No. 2 Thermo., ° F. | Percent CO <sub>2</sub> in air |      |
|-----------------|--------------------|-------------------------------|-------------------------------|--------------------------------|------|
|                 |                    |                               |                               | In                             | Out  |
| 1               | 120                | 122                           | 86                            |                                | nil  |
| 2               | 120                | 392                           | 149                           |                                | nil  |
| 3               | 120                | 527                           | 374                           |                                | nil  |
| 4               | 120                | 536                           | 482                           |                                | nil  |
| 5               | 120                | 527                           | 527                           |                                | nil  |
| 6               | 120                | 536                           | 536                           | 0.25                           |      |
| 7               | 120                | 717                           | 626                           |                                | 0.19 |
| 8               | 120                | 717                           | 707                           |                                | 0.12 |
| 9               | 120                | 717                           | 707                           |                                | nil  |
| 10              | 120                | 717                           | 707                           |                                | nil  |
| 11              | 120                | 887                           | 797                           |                                | nil  |
| 12              | 120                | 887                           | 887                           | 0.07                           |      |
| 13              | 120                | 887                           | 878                           | 0.14                           | 0.16 |
| 14              | 120                | 887                           | 887                           | 0.20                           | 0.47 |
| 15              | 120                | 887                           | 887                           | 0.42                           | 0.55 |
| 16              | 120                | 1,067                         | 987                           | 0.56                           | 0.75 |
| 17              | 120                | 1,067                         | 1,058                         | 0.54                           | 0.96 |
| 18              | 120                | 1,067                         | 1,067                         | 0.69                           | 0.66 |
| 19              | 120                | 1,067                         | 1,067                         | 0.63                           | 0.79 |
| 20              | 120                | 1,250                         | 1,202                         | 0.62                           | 0.89 |
| 21              | 120                | 1,250                         | 1,250                         | 0.24                           | 0.84 |
| 22              | 120                | 1,250                         | 1,250                         | nil                            | 0.81 |
| 23              | 120                | 1,250                         | 1,250                         | 0.17                           | 0.34 |
| 24              | 120                | 1,250                         | 1,250                         | nil                            | nil  |

The next two examples show the improvement when the method of the present invention is applied on a commercial scale.

## EXAMPLE IX

The conventional dehydrogenation unit was loaded with new calcium nickel phosphate-chromium oxide catalyst. Approximately 18,000 lb./hr. of air was passed through the butene furnace and into the reactors which were operated in parallel. A small amount of air was permitted to back around through the superheaters and was vented at a waste heat boiler. This warmed the steam lines and helped to prevent condensation in the lines when the steam was finally introduced. The temperature of the air to the reactors was raised to 340° F. in 1 hour and 20 minutes using only one burner on each side of the furnace which was used to heat the air. This temperature was maintained for 7½ hours and was then raised to 400° F. in a period of 1 hour and 20 minutes. After 2 hours and 20 minutes at this temperature, every thermocouple in both catalyst beds indicated a temperature greater than 225° F. At this point, the heating was continued with superheated steam from the furnace only. The calcium nickel phosphate-chromium oxide catalyst air start-up was successfully completed in a total elapsed time of 12½ hours.

## EXAMPLE X

The conventional dehydrogenation unit was loaded with new calcium nickel phosphate-chromium oxide catalyst. Air was introduced in the same manner as in Example IX and the temperature of the air to the reactors was raised to 500° F. in 4 hours and 20 minutes. This temperature was maintained for 6 hours and then raised to 520° F. in a period of 40 minutes. After 2½ hours at this temperature, every thermocouple in both catalyst beds indicated a temperature greater than 225° F. The heat-

ing was continued with superheated steam from the butene furnace. This calcium nickel phosphate-chromium oxide catalyst air start-up was successfully completed in a total elapsed time of 13½ hours.

Thus, using the process of the present invention the fresh calcium nickel phosphate-chromium oxide dehydrogenation catalyst may be ready for dehydrogenation in a period of about 13 hours, whereas the conventional methods result in a time lapse of about 48 hours.

In the process of the present invention it is very important that the temperature be controlled. It was found that, when the minimum temperature of the catalyst bed reaches 225° F. it is possible to use superheated steam instead of the heated air to heat the catalyst bed to its operating temperature and to remove the graphite from the surface of the catalyst pellets by means of heating the catalyst further with such superheated steam and adding a controlled amount of air. While it is, of course, possible to use a higher temperature providing no uncontrolled burning of the graphite occurs and hence possible destruction of the catalyst, the preferred maximum temperature of the inlet air is 600° F.

It is desirable to raise the temperature of the air to about 500° F. within the first two hours of the first admission of air, and the temperature should then be regulated to 550–580° F.

What I claim is:

1. In the process of commencing a reaction for the dehydrogenation of monoolefins having at least four carbon atoms in the olefinic chain using new calcium nickel phosphate-chromium oxide catalyst in the form of pellets which contain graphite, the improvement which comprises effecting the start-up of such catalyst by passing air at a maximum temperature of about 600° F. through such catalyst until the temperature of the catalyst bed is about 225°–450° F. and subsequently passing superheated steam at a temperature of 400° F.–1400° F. and a controlled amount of an oxygen-containing gas through said catalyst in order to oxidize said graphite and to heat said catalyst to the required dehydrogenation temperature.

2. In the process of commencing a reaction for the dehydrogenation of n-butylene to butadiene-1,3 using new calcium nickel phosphate-chromium oxide catalyst in the form of pellets which contain graphite, the improvement which comprises effecting the start-up of such catalyst by passing air at a maximum temperature of about 600° F. through such catalyst until the temperature of the catalyst bed is about 225°–450° F., and subsequently passing superheated steam at a temperature of 400°–1400° F. and a controlled amount of an oxygen containing gas through said catalyst in order to oxidize such graphite and to heat said catalyst to the required dehydrogenation temperature.

3. In the process of commencing a reaction for the dehydrogenation of monoolefins having at least four carbon atoms in the olefinic chain using new calcium nickel phosphate-chromium oxide catalyst in the form of pellets which contain graphite, the improvement which comprises effecting the start-up of such catalyst by passing air at a maximum temperature of about 600° F. through such catalyst until the temperature of the catalyst bed is about 225°–450° F., discontinuing the passage of air through said bed, passing superheated steam at a temperature of 400° F.–1400° F. through the catalyst bed until the temperature of the bed is about 900–1150° F. and continuing the passage of such steam while adding thereto a controlled amount of an oxygen-containing gas in order to oxidize said graphite.

4. In the process of commencing a reaction for the dehydrogenation of n-butylene having at least four carbon atoms in the olefinic chain using new calcium nickel phosphate-chromium oxide catalyst in the form of pellets which contain graphite, the improvement which comprises effecting the start-up of such catalyst by passing

air at a maximum temperature of about 600° F. through such catalyst until the temperature of the catalyst bed is about 225°-450° F., discontinuing the passage of air through said bed, passing superheated steam at a temperature of 400° F.-1400° F. through the catalyst bed until the temperature of the bed is about 900-1150° F. and continuing the passage of such steam while adding thereto a controlled amount of an oxygen-containing gas in order to oxidize said graphite.

## References Cited in the file of this patent

## UNITED STATES PATENTS

- 2,442,320 Britton et al. ----- May 25, 1948  
5 2,739,996 Pitzer ----- Mar. 27, 1956

## OTHER REFERENCES

- Britton et al. II, Ind. and Engr. Chem., vol. 43 (1951)  
pp. 2871-2874.